

July 4, 1944.

S. R. SHELMIRE ET AL

2,353,090

KNIT FABRIC AND METHOD OF MAKING THE SAME

Filed July 16, 1942

2 Sheets-Sheet 1



Fig. 1.



Fig. 2.

*Inventors*  
STANLEY R. SHELMIRE  
PAUL COOPER

*by their attorneys*

*Hawson and Hawson*

July 4, 1944.

S. R. SHELMIRE ET AL

2,353,090

KNIT FABRIC AND METHOD OF MAKING THE SAME

Filed July 16, 1942

2 Sheets-Sheet 2

NEEDLES



Fig. 3.

Fig. 4.

*Inventors*  
STANLEY R. SHELMIRE

PAUL COOPER

*by their attorneys*

*Howson and Howson*

Patented July 4, 1944

2,353,090

# UNITED STATES PATENT OFFICE

2,353,090

## KNIT FABRIC AND METHOD OF MAKING THE SAME

Stanley R. Shelmire and Paul Cooper, Laconia,  
N. H., assignors to Scott & Williams, Incorporated,  
Laconia, N. H., a corporation of Massachusetts

Application July 16, 1942, Serial No. 451,198

17 Claims. (CL. 66—202)

This invention relates to knitted fabrics and more particularly to a knitted fabric having elasticity regardless of whether or not it contains threads which are themselves elastic. In this specification the word "thread" will be used in its broad sense so as to include not only ordinary knitting yarns but also such filaments as glass thread, metal wire, etc. It is characteristic of the invention that two kinds of threads are used and that those two kinds of threads differ in their stiffness and flexing resilience.

In the accompanying drawings, we have illustrated on an exaggerated scale how our invention may be carried into effect. Merely for illustrative purposes to aid in the ready comprehension of the manner of interknitting the threads in interspersed courses, we have indicated in solid black the threads which are relatively stiff and resilient on flexure, while the pliable threads are indicated by outline.

In the drawings:

Figure 1 is a diagram of the interlacing of the threads in a piece of fabric knitted in accordance with our invention, the fabric being shown at rest; the words "needle" and "sinker" designating the relative positions of those elements in knitting the fabric;

Figure 2 is a similar diagram of the same piece of fabric partially stretched in a walewise direction;

Figure 3 is a similar diagram of the same piece of fabric fully stretched in a walewise direction;

Figure 4 is a diagram of the interlacing of the threads in a modified form of fabric in which a pliable yarn is knit in with the flexibly resilient 35

Figure 5 is a diagram of the interlacing of the threads of a fabric made in accordance with our invention in which the course sequence of the threads is different from that of Figures 1 to 4.

Heretofore when it was desired to make a knitted fabric which was elastic, it was customary to knit the fabric of a yarn which could itself stretch longitudinally and rely on that elasticity to give elasticity to the fabric. Such elastic yarns are principally rubber and its substitutes. All such yarns are fragile and short-lived, and under present war conditions are unobtainable for civilian use. They are not stiff and could not be used ordinarily to give our novel fabric. 50 We have discovered that under certain conditions it is possible to make a knitted fabric which is elastic, due, not to the ability of the threads to stretch and return to their normal lengths, but to other factors. In other words the elasticity of 55

our novel fabric is not dependent on the yarn being "elastic" in the sense that the yarn can stretch longitudinally and return to its normal length when released. In many cases our fabric is preferably made from yarns which actually cannot stretch.

One of the threads 10 used in our novel fabric must be relatively resilient on flexure, and another thread 20 in the fabric must be relatively pliable. It is the interaction of these two types of threads assembled in the manner to be described which produces our elastic fabric. The flexibly resilient or spring-like thread may be a metal wire or strip such as a spring, cotton, rayon, a synthetic thermoplastic yarn, regardless of whether it is elastic or inelastic, or it may be any other natural or synthetic yarn which is flexibly resilient and has the other necessary qualities hereinafter set forth. We have found, for example, that the synthetic thermoplastic yarns formed of vinylidene chloride resins and known as "Saran" and those formed of fibre-forming polymeric amides known as "Nylon" are suitable for use in our fabric.

25 The other or non-resilient yarn of our novel fabric must be pliable and not too resistant to sliding at points where it contacts the other threads. It is preferably a fibrous thread. The resilient and non-resilient threads must be formed into loops in alternation. One factor in the production of the elasticity of the fabric is the drawing of a stitch or course of stitches of the resilient thread through a stitch or course of stitches of the pliable thread. Thus for example in Figures 1 to 3 we have shown a fabric in which one alternate course 11 knit of the resilient thread 10 is interspersed with one intermediate course 21 knit of the pliable thread 20. That is the preferable course arrangement, but it should be understood that the alternation need not be 1 x 1.

45 We will now explain in what manner it is believed the resilient and non-resilient threads interact to give elasticity to the fabric. When the resilient thread is knit it is constantly straining toward a straight position and the result is that the stitch formed of this resilient thread is quite wide (see Fig. 1). The center or top of the needle wales is at the point marked "needle." It will be observed in Fig. 1 that the legs of the needle wales are not vertical but separate or diverge from the tops of the wales at a wide angle so that the loops are opened up laterally. The threads do not assume this particular position

completely until after they have passed the knocking-over point in the knitting machine.

Figures 1, 2 and 3 of the drawings illustrate the interaction of the threads as the fabric is pulled walewise from its relaxed condition (Fig. 1) to a partially extended condition (Fig. 2) and finally to a fully extended condition (Fig. 3). It will be observed that as the fabric is stretched walewise the fabric and the stitches become narrower and deeper. Thus the top portion 22 of the pliable thread 20 of the left-hand needle wale in Fig. 1 has become shorter, as shown at 23 in Fig. 2. The legs 24 of this needle wale in Fig. 1 are quite short, while in Fig. 2 they are distinctly longer, as shown at 25. The sinker wale 26 of this same yarn is also starting to shorten up slightly in Fig. 2. In Fig. 3 the top of the needle wale is of only the width of ordinary fabric, as shown at 28, while the legs 30 of this needle wale in this figure are of the length of such legs in normal fabric.

The walewise stretch of the fabric pulls the legs 12 of the resilient needle wales together and causes the thread to bow out in a needle wale shape (Fig. 3) more usual than that of Figs. 1 and 2. It will be noted that the resilient thread 10 in the stretched fabric (Fig. 3) is more bowed than the non-resilient thread 20, which latter is more aptly described as sharply bent than resiliently bowed.

When the fabric is at rest it is necessary for the legs of the needle wales not to be in contact with each other. Unless this is true, there is no room for the stitch to bend resistively and thereby to have elasticity in the fabric. The pliable thread stitches should be knitted loosely to take full advantage of this effect.

If the resilient thread being used is a synthetic thermoplastic thread, it has been found further advantageous to treat the fabric after it is knit. This treatment consists of pressure and heat. One purpose of the pressure is to improve the appearance of the fabric, but it has also been found when the fabric is subjected to heat and pressure, that the elasticity of the fabric is slightly increased. The purpose of the application of heat is to "set" the resilient thread in its new position. As is well known, when a synthetic thermoplastic yarn is set by heat, the shape or convolutions of the yarn at the time of heating become its normal or strain-free condition. Thereafter the thread resists any attempt to change it from that position instead of the straight position which was the normal or strain-free condition of the thread when it entered the knitting machine. As indicated, this combined pressure and setting of the thread by heat widens the fabric slightly and increases the amount of its elasticity. It also seems to increase slightly the ability of the fabric to return to normal after stretch and its resistance to stretch.

The effect of this wide or opened-out course of stitches of the resilient thread on the non-resilient thread is to make the stitches of non-resilient thread shallow and wide. When drawn in the knitting machine this stitch of non-resilient thread at first was of normal length in a walewise direction. As soon as the resilient thread got away from the knitting point it tended to straighten, thus broadening the sinker and needle wales of the non-resilient thread and decreasing the length of the stitch. In this way the stitch of pliable thread becomes shallow and wide. When the threads are in the position shown in Fig. 1, the fabric is of its maximum

width and minimum length and it has practically no elasticity in a coursewise direction. This is its normal or relaxed condition. However, the fabric has a large amount of stretch in a walewise direction. It will also be noted that the stitches of resilient thread are shallower than if they had not moved after being knitted. Thus the interspersing of the resilient and non-resilient threads during the knitting produces a wide fabric but one that has shallow stitches and is short in a walewise direction.

From the description thus far given it will be obvious that it is immaterial whether the resilient thread is also elastic in its length or not—at least as far as concerns the elasticity of the fabric due to the interspersing of the resilient and non-resilient stitches in the knitted fabric.

The above-mentioned changes in shape of the stitches of non-resilient thread necessitate a sliding of the pliable thread 20 on the resilient thread 10. There also is sliding of the resilient thread on the pliable thread. It has been found that when both resilient and non-resilient threads have a large number of filaments in them, the sliding is so interfered with that the elastic character of the fabric is largely lost. For this reason we have found it advisable to make the resilient thread of very few filaments and preferably a monofilament and of large cross-section, such as is found in plastic yarns. The large cross-section presumably also plays its part in the stiffness and flexible resilience of the yarn. In this form the synthetic thermoplastic threads known as "Saran" and "Nylon" are smooth and slide well. Any combination of threads which permits easy sliding of the threads on each other will be satisfactory for our fabric, provided the contrasting characteristics as to resilience and pliability are present. However, if the fabric is to be used on or adjacent to human flesh, it probably will be inadvisable to use a thread like piano wire because of the danger of a broken thread causing a scratch.

We have discovered that our elastic effect in the fabric can be obtained to a modified extent if groups of one, two or three courses of resilient or non-resilient thread are together. Beyond that point most of the effect is lost. The more courses of non-resilient thread between the resilient thread, the less elasticity, although under certain conditions two courses may give more stretch than one. The interlacing of one resilient loop with another does only a little to increase the resilience of the fabric. While the interlacing of one stitch of non-resilient thread with another non-resilient thread increases the stretch of the fabric slightly, it also tends to reduce the ability of the fabric to return to its original size when released. Such a construction is shown in Fig. 5, where the alternation is two courses of non-resilient yarn 28 and one of resilient yarn 10. This gives more of the pliable thread to be pulled by the resilient thread.

If desired, the harsh feeling of some of the resilient thread available for use in our fabric can be largely eliminated by knitting a rayon or other softer thread 40 with the resilient thread 10 (Fig. 4). The inelastic thread is caused to cover the elastic by the method set forth in the John Lawson Patent 2,009,361, dated July 23, 1935. The covering thread 40 can be the same as the pliable fibrous thread 20 or not, as desired.

If desired, the fabric can be knit in a knitting machine where there are two sinkers between

two adjacent needles, as indicated for example in Fig. 1. This has the effect of producing a long sinker wale and increasing the extent to which the fabric can be stretched in a walewise direction. Similarly, any lengthening of the needle wale would tend to increase the separation of the legs of the needle wale.

If the elasticity of the fabric exhibits fatigue, the fabric can be washed and reset by heat and pressure, whereupon it resumes all its original elasticity and strength.

We claim:

1. Knitted fabric comprising threads of different character as to stiffness and resilience, in which groups of one to three courses containing a relatively stiff but flexibly resilient thread are alternated repeatedly with groups of one to three courses containing a relatively pliable thread, said flexibly resilient thread being present in stitches opened out whereby said stitches contract the fabric in a walewise direction, giving the fabric elasticity in that direction.

2. Fabric knit of groups of from one to three courses of a stiff but flexibly resilient thread interknit in repeated succession with groups of from one to three courses of a pliable thread, the resilience of the stiff thread opening the stitches of said thread laterally and contracting the stitches walewise and making the fabric elastic in that direction.

3. In weft knit fabric in which threads of different characteristics are present for the purpose of giving elasticity to the fabric, a relatively stiff and flexibly resilient thread knit in alternate courses, in combination with a relatively pliable thread knit in the intermediate courses, the resilient thread opening its stitches laterally and tending to straighten out and thereby shorten both resilient and pliable stitches in the walewise direction, contracting the fabric and giving it elasticity in that direction.

4. Weft knit fabric in which relative differences in stiffness and flexing resilience of thread are used to give elasticity to the fabric, there being a relatively stiff and flexibly resilient thread knit in alternate courses, in combination with a relatively pliable thread in the intermediate courses, the resilient thread widening its own stitches and those of the pliable thread, shortening the fabric and making it elastic in a walewise direction.

5. Weft knit fabric in which relative differences in stiffness and flexing resilience of threads are used to give elasticity to the fabric, the fabric at rest containing one or two courses of a relatively stiff and flexibly resilient thread formed in stitches with the legs of the needle wales bent apart due to the resilience of the thread, in combination with a relatively pliable thread in one or two courses interspersed with the resilient thread, the stitches of the pliable thread making wide and shallow stitches due to the spreading of the legs of the needle wales of the resilient thread, said legs being pulled together against the resilient power of that thread when the fabric is stretched in a walewise direction, so that the fabric is elastic in that direction.

6. Knitted fabric composed of alternate courses of threads some of which have different characteristics arranged in courses in repeated succession, there being present in one type of course a stiff and flexibly resilient thread of a smoothness permitting the thread interlaced with it from adjacent courses to slide thereon, the intermediate courses containing a more pliable

and non-resilient thread, said resilient thread, tending to straighten out, forms stitches laterally opened out and contracts the fabric in a walewise direction, thereby giving the fabric elasticity in that direction.

7. Weft knit fabric having extra elasticity in a walewise direction in which the threads in alternate courses have stiffness and resilience to bending and the threads in the intermediate courses have less resilience to bending, said more resilient stitches tending to straighten out, opening the stitches laterally and pulling the less resilient thread stitches into a shallow, wide shape, with the result that a reserve for increase in length of the fabric in case of tension thereon is created.

8. In a weft knit fabric containing alternate courses in which threads are present having different characteristics, the combination of a thermoplastic thread having stiffness and flexible resilience in one course and a pliable thread in the other course, said two threads being interknit, the thermoplastic thread being "set" with its stitches laterally opened out whereby on walewise tension the legs of the resilient needle wales will come together and the stitches of the more pliable thread interlaced throughout those legs become narrower and longer and the fabric stretches in the walewise direction.

9. Knitted fabric composed of alternate courses containing at least pliable thread in one course and a stiff and flexibly resilient thermoplastic thread in the other, said thermoplastic thread being present in stitches laterally opened out, whereby the flexibly resilient thread permits the fabric to be stretched walewise and its resilience contracts the fabric again when the tension is released.

10. Knitted fabric composed of alternate courses containing at least pliable fibrous thread in one course and a stiff and flexibly resilient thermoplastic monofilament thread of large cross-section in the other, said thermoplastic thread being present in stitches laterally opened out, whereby the flexibly resilient thread permits the fabric to be stretched walewise and its resilience contracts the fabric again when the tension is released.

11. Knitted fabric having extra elasticity in a walewise direction composed of alternate courses in which there are present stiff and flexibly resilient thread in one course and pliable thread in the other, the stitches in which these threads are present being interlaced with each other in alternation in a walewise direction, the stitches of the resilient thread being laterally opened out thereby forcing all the stitches of the fabric to be wide and shallow, whereby the tendency of the resilient thread to straighten out provides elasticity in the walewise direction in the fabric.

12. A method of making weft knit fabric having extra elasticity in a walewise direction, composed of knitting one or more courses of a relatively pliable and flexibly non-resilient fibrous thread in repeated succession to one or more courses of a thermoplastic thread resilient to bending, allowing the resilient thread to pull the non-resilient stitches into a wide shallow shape and setting the thermoplastic thread while the fabric is in this condition.

13. In a method of making knitted fabric having extra elasticity in a walewise direction, the steps of knitting alternate courses of relatively stiff and flexibly resilient thermoplastic thread

and relatively pliable thread while forming extra width sinker wales and allowing the resilience of the thermoplastic thread to hold the pliable thread in shallow wide shape, and thereafter setting the thermoplastic thread in this slightly bent position, whereby tension on the fabric in a wale-wise direction tends to pull the legs of the thermoplastic stitches into more normal parallel formation against the resilience of the thermoplastic thread with resultant extension of the fabric walewise. 10

14. In a method of making knitted fabric having extra elasticity in a walewise direction, the steps of knitting courses of relatively stiff and flexibly resilient thermoplastic thread in alternation with the knitting of courses of relatively pliable thread while allowing the stitches of the latter thread to be formed loosely, thus permitting the legs of the needle wales of the resilient thread to spring apart and form the pliable thread into shallow wide stitches, whereby tension on the fabric in a walewise direction tends to pull the legs of the needle wales of the resilient thread into more parallel formation against the resilience of the thread, thereby permitting the fabric to stretch in a walewise direction and return to its normal length when the tension is released. 20

15. Weft knit fabric composed of alternate courses of threads of different characteristics, alternate courses being knitted of relatively stiff, 30

flexibly resilient monofilament thread, in combination with a more pliable covering thread, and the alternate courses having in them a relatively pliable thread knit loosely, said resilient thread being present in stitches laterally opened out whereby the resilient thread holds all the stitches of the fabric in a wide shallow shape and resists, resiliently, efforts to stretch the fabric in a walewise direction, the monofilament and pliable threads sliding on each other to make the necessary changes in the shapes of the stitches as the fabric is stretched and relaxed. 15

16. Knitted fabric composed of alternate courses containing at least pliable thread in one course and a Saran thread in the other, said Saran thread being present in stitches laterally opened out, whereby the Saran thread permits the fabric to be stretched walewise and its resilience contracts the fabric again when the tension is released. 25

17. In a fabric knit of relatively pliable thread, a relatively stiff and flexibly resilient thread knit in the alternate courses, said resilient thread opening its stitches laterally and thereby shortening both resilient and pliable thread stitches in the walewise direction to contract the fabric and give the fabric elasticity in the walewise direction. 35

STANLEY R. SHELMIRE.  
PAUL COOPER.